

June 10, 1958

J. ROCKOFF

2,837,775

TEXTILE COT

Filed July 19, 1952



Fig. 1



Fig. 2

INVENTOR.  
JOSEPH ROCKOFF

BY *Joseph Rockoff*  
ATT'Y.

1

2,837,775

## TEXTILE COT

Joseph Rockoff, Dayton, Ohio, assignor to The Dayton Rubber Company, a corporation of Ohio

Application July 19, 1952, Serial No. 299,841

9 Claims. (Cl. 19—143)

The present invention relates to textile machine units, and more particularly, to cots or roll covers for spinning rolls or other rolls used in the drafting or spinning of textile fibers.

A textile roller as used in present day cotton and spinning machines comprises a metal core or arbor having a sleeve-like roll cover known as a cot, surrounding the core. In the past these covers have been made of leather, cork compositions, or certain types of rubber compounds especially adapted for this purpose.

At one time most textile cots were made of leather, but this material proved to be unsatisfactory for use on cotton machines which work at relatively high speeds, due to stretch, lack of uniformity, short life, and relatively poor drafting properties particularly in connection with lapping up and eyebrowning. In recent years cots have been made of synthetic materials which show considerably longer life than leather and have greater resistance to lapping up and eyebrowning and have, in general, proved to be a satisfactory substitute for leather.

Despite the improved characteristics which have been imparted to textile cots by the use of certain types of synthetic rubber, these cots do not function perfectly under all conditions and for all types of fibers. Some of the newer types of cots, although considerably improved over leather, still exhibit a tendency toward eyebrowning. This condition results from the failure of the cot to carry short fibers or clearer waste to the top clearer in order to gather properly. Instead, these short fibers collect at the outside edge of the top clearer and hang down over the roll. This condition is called eyebrowning, and the mass of fibers which hang down is called an eyebrow. As the size of the eyebrow increases, it will touch the yarn and bunches of short fibers will become intermingled with the yarn thus impairing its quality.

It has been found that cork may be used as a roll covering or in admixture with rubber with a certain degree of success as a textile drafting material. However, the use of cork has been found to have certain disadvantages, among which are a certain degree of hygroscopicity, poor resistance to indenting or marking as a result of the contact with the fibers, and a tendency to become slick and change its drafting properties after a period of use. Such cots are also found to be affected by light resulting in the change in drafting properties. As a result, frequent grinding is necessary in order to renew the surface.

In accordance with the present invention, applicant has now discovered that improved drafting properties are obtained by the incorporation of minor proportions of ground particles of the soft fibrous shells of certain types of nuts. These shells must be of a soft, porous and fibrous structure, the most common examples of which are the hulls of peanuts and the shells of almonds. These shells are ground to a desired particle size and incorporated into a suitable rubber compound by milling or

2

any other suitable manner, prior to formation of the cot by extrusion or otherwise.

The appended drawings illustrate a typical cot construction of the present invention.

5 In the drawings:

Figure 1 shows a view in elevation partly in cross section of a conventional type of double cot mounted on an arbor.

Figure 2 illustrates in cross section an enlarged view 10 of a portion of the cross section of the cover shown in Figure 1.

In the drawings the double arbor is represented by 15 10, each side of the arbor having a roll cover 11 and 11a mounted thereon. The particles 13 which are embedded in the composition, are exposed at the surface of the roll and are also shown embedded in the roll compound 11 in Figure 2.

In the fabrication of the cot referred to, the nut hulls 20 are ground to a predetermined size and incorporated in the unvulcanized rubber compound in the desired proportions along with vulcanizing and other compounding ingredients. The mixture is then extruded in a tubular form, placed on a core, rag wrapped, and vulcanized. After vulcanization, the rag wrap is removed and the 25 resulting product ground down to the desired size. After this, the tube is cut to the desired lengths and the cots mounted on the arbor. A finish grind may be used before the cot is placed in operation. The preferred type of synthetic rubber with which this material is incorporated is an oil-resistant copolymer of the butadiene-acrylic nitrile type; also known as Buna-N, perbunan, GR-A, or by other well-known terms used in the trade. While 30 the particle size and range of proportions of the nut shell material may vary considerably over a wide range, it has been found that certain particle sizes and proportions 35 are of greater importance in obtaining optimum results. The particle size is generally preferred to be in the range of about 20 to 60 mesh, and the range of proportions is generally preferred to be a range of about 20 to 125 parts per 100 parts of rubber by weight based 40 on the rubber in the compound.

The following example will illustrate a typical cot compound of the type described above:

|                                                                | Parts of weight |
|----------------------------------------------------------------|-----------------|
| Perbunan (74% butadiene 26% acrylo-nitrile emulsion copolymer) | 100             |
| Plasticizer and tackifier phenol-formaldehyde resin (Bakelite) | 10-20           |
| 50 Sulfur                                                      | 5               |
| Accelerator (mercaptobenzothiazole or the like)                | 1-2             |
| Zinc oxide                                                     | 8-12            |
| Clay filler                                                    | 15-35           |
| Diphenylguanidine                                              | 0.25            |
| 55 Ground peanut shells particle size 40 mesh                  | 50              |

Compounds corresponding to the foregoing recipe were 60 mixed, extruded, vulcanized and made into cots in the manner described above. The resulting cots were then placed on an experimental spinning frame drafting cotton and rayon fibers in comparison with other cots of the same composition but without the peanut shells. The new composition of the present invention was found to outperform the other compound with respect to lack of 65 eyebrowning and lapping up, particularly in the drafting of synthetic fibers. Other proportions and particle sizes of the shells are also effective as are ground almond shells.

I claim:

70 1. A textile fiber drafting cot having a working surface composed of vulcanized oil-resistant synthetic rubber having intimately incorporated therewith a minor pro-

portion of particles of soft, porous, fibrous nutshells, said particles being exposed at said cot surface.

2. A textile fiber drafting cot having a working surface composed of vulcanized oil-resistant synthetic rubber having intimately incorporated therewith a minor proportion of particles of ground up peanut shells, said particles being exposed at said cot surface.

3. A textile fiber drafting cot having a working surface composed of vulcanized oil-resistant synthetic rubber having intimately incorporated therewith a minor proportion of particles of ground up almond shells, said particles being exposed at said cot surface.

4. A textile fiber drafting cot having a working surface composed of vulcanized oil-resistant synthetic rubber having intimately incorporated therewith a minor proportion of particles of soft, porous, fibrous nutshells, wherein the particles range in size from about 20 mesh to about 60 mesh and are incorporated in the proportion of about 20 to 125 parts of the shell per 100 parts of synthetic rubber by weight, said particles being exposed at said cot surface.

5. A textile fiber drafting cot having a working surface composed of a vulcanized oil-resistant butadiene-acrylic nitrile copolymer having intimately incorporated therewith a minor proportion of particles of soft, porous, fibrous nutshells, said particles being exposed at said cot surface.

6. A textile fiber drafting cot having a working surface composed of a vulcanized butadiene-acrylic nitrile copolymer having intimately incorporated therein a minor

portion of particles of peanut shells, said particles being exposed at the surface of the cot.

7. A textile cot according to claim 6 wherein the peanut shells have a particle size of about 20 to 60 mesh and are incorporated in the proportion of about 20 to 125 parts per 100 parts of vulcanized butadiene-acrylic nitrile copolymer by weight.

8. A textile cot according to claim 6 wherein the peanut shells have a particle size of about 40 mesh and are incorporated in the proportion of about 50 parts per 100 parts of vulcanized butadiene-acrylic nitrile copolymer by weight.

9. A textile fiber drafting cot having a working surface composed of a vulcanized butadiene-acrylic nitrile copolymer having intimately incorporated therein a minor proportion of particles of almond shells, said particles being exposed at the surface of the cot.

References Cited in the file of this patent

UNITED STATES PATENTS

|           |             |               |
|-----------|-------------|---------------|
| 2,373,698 | McGeary     | Apr. 17, 1945 |
| 2,414,803 | D'Alelio    | Jan. 28, 1947 |
| 2,450,410 | Baymiller   | Oct. 5, 1948  |
| 2,467,214 | Luaces      | Apr. 12, 1949 |
| 2,570,935 | Freedlander | Oct. 9, 1951  |
| 2,585,219 | Boyle       | Feb. 12, 1952 |
| 2,645,587 | Williamson  | July 14, 1953 |

FOREIGN PATENTS

|        |               |         |
|--------|---------------|---------|
| 15,988 | Great Britain | of 1915 |
|--------|---------------|---------|